

Nov. 7, 1933.

J. F. BRIGGS ET AL.

1,934,618

## TREATMENT OF CELLULOSE DERIVATIVES

Filed Aug. 2, 1929

FIG. 3.

FIG. 1.



FIG. 4.



FIG. 5.



FIG.-2-

JOHN F. BRIGGS

ROBERT P. ROBERTS

ROBERTS  
Inventors

INVENTOR'S  
Signature

I. Seligson & C. W. Levinson  
Inventors  
Attorneys

## UNITED STATES PATENT OFFICE

1,934,618

## TREATMENT OF CELLULOSE DERIVATIVES

John Frederick Briggs and Robert Pierce Roberts,  
Spondon, near Derby, England, assignors to  
Celanese Corporation of America, a corpora-  
tion of Delaware

Application August 2, 1929, Serial No. 382,907,  
and in Great Britain August 13, 1928

## 30 Claims.

(Cl. 18—8)

This invention relates to the manufacture of artificial silk and other filaments or threads from solutions of cellulose acetate or other cellulose derivatives, and particularly to their manufacture by the dry or evaporative method.

It is, of course, of the utmost importance to ensure that filaments of uniform character can be produced in any desired number of cells, and that any particular type of filament can be produced at will by varying the conditions of operation of the spinning plant. By the use of the means described in U. S. Patent No. 1,541,104, filaments and threads of high quality and uniformity are produced by controlling the amount 10 of evaporative medium, e. g. air, passing through each cell and by enabling a uniform flow to be obtained in any desired number of cells, for, while numerous variations may be introduced in the control and operation of the spinning plant, it 15 has been found of particular importance to ensure regularity of the flow of evaporative medium passing through the cells of the plant. Further, while the evaporative medium may be introduced at the top, or bottom, or elsewhere into the cell, and may 20 be introduced already heated or not, the above-mentioned requirements as to regularity of flow and uniformity of flow as between all the cells must always be observed if uniform filaments or 25 threads of high quality are to be obtained, and the means described in U. S. Patent No. 1,541,104, for 30 controlling the flow may be used for this purpose in all these cases.

Further means for controlling the spinning operation are described in U. S. Patent application 35 S. No. 236,448 filed 29th November, 1927, which describes collector devices adapted to utilize the full evaporative capacity of the evaporative medium by constraining practically the whole of it to pass through the immediate vicinity of the 40 nozzle, these collector devices enabling a stricter control to be exercised over the cross-section of the filaments, and allowing flat, semi-flat, or substantially rounded filaments to be obtained at will.

It has now been found that the uniformity and 45 character of the filaments or threads can be controlled to a degree hitherto unattainable by introducing an evaporative medium into the spinning cell in the vicinity of the spinning jet. The evaporative medium thus introduced is preferably directed into proximity to the filaments issuing 50 from the jet, and it may be introduced into the cell at the level of the jet face or at some distance behind or in front of the jet face. The medium may be heated or not, as desired and may contain 55 if desired, vapours, such as for example, vapours

of the solvent or solvents used in the spinning solution, though, preferably, the evaporative medium is introduced alone into the cell.

Any suitable device may be employed for the introduction of the evaporative medium. Thus, 60 for example, a perforated or slotted tubular ring, a straight or curved perforated or slotted pipe, a jet or jets, or other orifice or orifices, may be arranged at the desired level in the cell with respect to the level of the spinning jet or nozzle. 65 The direction taken by or imposed on the evaporative medium introduced by the ring, tube, or other device may be the same as that of the issuing filaments, or may be opposed, normal, or otherwise arranged with respect thereto, while the 70 medium is with advantage applied symmetrically with respect to the bundle of filaments. Thus with a circular bundle of filaments, or series of concentric circular bundles of filaments the evaporative medium is advantageously caused to flow 75 through a space coaxial with the bundle or bundles of filaments.

The medium may be introduced in an amount which may be any desired proportion of the total 80 volume of solvent-laden medium drawn out of the chamber or cell, and, in order to control the admission of the medium, the pipe, tube, or other conduit employed therefor is preferably provided with control means similar to those described in U. S. Patent No. 1,541,104 with reference to the 85 draw-off from the cells, such means comprising a throat or constriction which is associated with a flow meter and a valve, all the individual chambers or cells of an installation being similarly 90 provided to ensure that the same conditions as to the introduction of the medium apply to all the chambers or cells, for the purpose of obtaining a uniform grade of filaments. In order to secure uniformity of flow of the evaporative medium in all the cells, it is important that the 95 draw-off from the cells also be controlled in the manner described in the above-mentioned U. S. Patent No. 1,541,104. The draw-off from the cells and the admission of evaporative medium to the vicinity of the spinning jets may be so controlled that the amount of medium introduced in the vicinity of the jets can vary from a relatively 100 small proportion of the total amount of evaporative medium to a relatively large proportion or even the total thereof.

Pressure may be employed to effect the introduction of the medium to the vicinity of the jets, though the suction of the draw-off devices may be used to aspirate the desired amount of medium, particularly where the admission conduit 110

for such medium is provided with a throat or constriction as described above.

The medium introduced in the vicinity of the jets may be heated before its introduction, and any suitable means may be employed to impart the desired degree of heat thereto, but, on the other hand, cold or comparatively cold medium may be introduced into the cell if desired.

The invention is applicable to any dry-spinning process or apparatus. For example, it may be used in connection with dry-spinning processes in which the spinning solution is extruded downwardly into an upwardly moving current of evaporative medium, or upwardly into a downwardly moving current, or in any other processes in which solidification of the filaments is effected by means of evaporative medium.

When the invention is employed in conjunction with spinning processes in which the filaments are extruded into a current of evaporative medium, devices may be employed whereby the whole or substantially the whole of the current of evaporative medium is constrained to pass through the immediate vicinity of the filaments moving through the cell, for example, such devices may extend across the whole width of the cell with the exception of an area substantially occupied by the filaments, and may be similar to the devices for constraining the evaporative medium to pass through the immediate vicinity of the filaments issuing from the jet or nozzle described in U. S. application S. No. 236,443. Further the chambers or cells may be of the type wherein the end remote from the jet or nozzle is open to the atmosphere of the spinning room, or wherein a relatively large number of jets or nozzles are arranged in each chamber or cell, as described in U. S. Patent applications S. Nos. 311,213 and 311,214 filed 8th October, 1928.

Where the evaporative medium which is to be introduced according to the invention is desired to contain a proportion of solvent or other vapours, the vapours may be introduced by admixture or by passing the medium through a moistening chamber, or by mixing it with solvent-laden medium, for example, solvent-laden medium withdrawn from the cell.

Several embodiments of the invention are illustrated in the accompanying drawing with reference to the downward spinning of artificial filaments, but it is to be understood that the following description is given by way of example only, and is in no way illustrative.

Fig. 1 shows a perspective view of one arrangement according to the invention, in which additional medium is introduced by means of perforated or slotted tubes;

Fig. 2 shows, in section, several alternative forms of a perforated or slotted tube;

Fig. 3 shows a form of device for use in connection with line jets;

Fig. 4 is a section on the line 4—4 of Fig. 3, and

Fig. 5 is a vertical section of a spinning cell, and illustrates means for controlling the amount of additional medium introduced into the cell, and the amount of solvent-laden evaporative medium drawn off from the cell.

Referring to Fig. 1, the jets 6 arranged for downward spinning are supported by the filter chambers 7, the upper portions of the chambers 7 being shown broken away for sake of clearness. A tubular ring 8 surrounds the axis of each chamber 7 and a pair of rings is connected by a tube 9. Each ring 8 may be at the level of the jet 6 or above or below such level. The supply pipe 10

is connected to the tube 9 and is connected to any suitable source for the supply of evaporative medium to the rings 8. It will of course be understood that instead of the rings 8 being connected in pairs to a common supply pipe, each ring may have its own supply pipe, or any other suitable number of rings may be connected to a single pipe.

Referring now to Fig. 2, (a) shows perforations or slots 11 on the under side of the ring 8, this position of the perforations being preferred when the ring 8 is arranged some distance above the level of the nozzle 6; (b) shows perforations 12 from which evaporative medium is directed substantially radially inwardly from the ring 8, and in (c) perforations 13 direct additional medium inwardly and somewhat downwardly from the ring 8. The forms (b), (c), are preferred when the ring 8 is at or about the level of the nozzle 6 or below the level of the nozzle 6. Instead of the perforations 12, 13 shown in Figs. 2 (a) and 2 (b), slots 12<sup>a</sup>, 13<sup>a</sup> may be employed. Likewise, a continuous slot may be formed round the rings 8, affording an annular passage for the evaporative medium. By the employment of any of the above described forms of perforated or slotted ring, the evaporative medium is directed into proximity to the filaments 14 issuing from the nozzles.

In Figs. 3 and 4, a perforated tube 15, of U-105 form, is connected by a pipe 16 to a supply of evaporative medium, and is so arranged with respect to a line jet 17 that slots or perforations 18 in the two limbs of the tube direct the medium into the vicinity of the filament 19 issuing from the jet 17. The slots or perforations 18 may cause the evaporative medium to be directed inwardly towards the filaments or somewhat upwardly or downwardly as well as inwards, or upwardly or downwardly parallel to the filaments. As has 115 been described with reference to Fig. 1, the tube 15 may be arranged at the level of the jet 17, or at some distance above or below the jet.

In Fig. 5, a perforated or slotted ring or tube 20 is connected by a pipe 21 to a supply header 120 22, the header 22 serving to deliver evaporative medium to any desired number of devices 20. For the purpose of controlling the amount of medium introduced into the cell 23 through the ring or tube, and particularly for enabling uniform amounts to be introduced to a number of cells required to produce a uniform grade of filament, a valve 24 is inserted in the pipe 21 and is operated in accordance with the reading of a flow meter 25, which is connected to the pipe 21. 130

For the purpose of controlling the amount of solvent-laden evaporative medium drawn from each cell 23, and particularly for obtaining a uniform draw-off from a number of cells in which uniform filaments are to be produced 135 simultaneously, control means such as those described in U. S. Patent No. 1,541,104 may be employed, as shown in Fig. 5. The evaporative medium is drawn off by suction through a pipe 26 under the control of a valve 27 and passes into a header 28. A flow meter 29 inserted in the pipe 26 between the valve 27 and the inlet 30 of the pipe enables the flow to be observed. The inlet 30 of the pipe 26 is arranged at the upper end of the cell 23 at a higher level than the jet face. 140

Heating of the evaporative medium introduced by the ring, tube, or other member may be effected, if desired, by means of heating devices arranged inside or outside the cell. For example, the connection of the ring, tube or the like to 145

- the source of evaporative medium (e. g. the pipe 10) may pass through the whole or part of the length of the cell before reaching the ring, tube, or the like.
- 5 According to the invention, uniform filaments of any required cross-section may be produced and by suitably controlling the temperature conditions in the cell, the quantity of evaporative medium passing therethrough, and the speed of the filaments, and/or of the evaporative medium, filaments of hollow cross-section may be obtained.
- 10 The invention may be applied to any type of cell or chamber for use in spinning by the dry or evaporating method, whether the cells are of relatively small or relatively great cross-section, whether circular in section or otherwise, or whether each cell contains one or other small number of jets or nozzles or a relatively large number of jets or nozzles. Also, where a current of evaporative medium is passed through the cell and is to be heated, such heating may be effected outside the cell, or inside by jackets surrounding the whole or a part of the length of the cell, by a coil or coils inside the cell, by banks or other arrangement of pipes extending through several cells, or by any other suitable means, control means being preferably provided whereby uniform or regulated variations in temperature may be effected along the height of the cell.
- 15 Filaments or threads produced according to the invention may be wound, or twisted and wound continuously with their production, for instance, by submitting them to a cap-spinning operation as described in U. S. Patent application S. No. 615,682 filed 29th January, 1923, such operations preferably being carried out outside the cell or chamber in which the filaments or threads are produced. Further the filaments or threads may be subjected to any desired operations such as moistening, lubricating, stretching, or sizing at any suitable point in their travel to the winding, or twisting and winding devices.
- 20 While the invention is particularly applicable to the production of filaments or threads having a basis of cellulose acetate, it may also be used in the manufacture of filaments or threads from solutions containing cellulose formate, propionate or butyrate, or thiocarbamic or alkoxy-alkacetyl esters of cellulose, or methyl, ethyl or benzyl cellulose, or the corresponding condensation products of cellulose and glycols or other polyhydric alcohols, or other substitution derivatives of cellulose that are capable of being formed into artificial filaments or threads by dry or evaporative methods.
- 25 What we claim and desire to secure by Letters Patent is:—
1. A process for the production of artificial filaments comprising extruding a spinning solution into a spinning chamber, introducing evaporative medium into the immediate vicinity of the filaments substantially at the point of extrusion, and withdrawing at least part of the evaporative medium entering the chamber at a point substantially at least as near the spinning end of the chamber as the point at which said introduction of evaporative medium is effected.
- 30 2. A process for the production of artificial filaments comprising extruding a spinning solution into a spinning chamber, introducing the whole of the evaporative medium required into the immediate vicinity of the filaments substantially at the point of extrusion, and withdrawing at least part of the evaporative medium entering the chamber at a point substantially at least as near the spinning end of the chamber as the point at which said introduction of evaporative medium is effected.
- 35 3. A process for the production of artificial filaments comprising extruding a spinning solution into a spinning chamber, introducing the whole of the evaporative medium required into the immediate vicinity of the filaments substantially at the point of extrusion, and withdrawing at least part of the evaporative medium entering the chamber at a point substantially at least as near the spinning end of the chamber as the point at which said introduction of evaporative medium is effected.
- 40 4. A process for the production of artificial filaments comprising extruding a spinning solution into a spinning chamber, introducing the whole of the evaporative medium required into the immediate vicinity of the filaments substantially at the point of extrusion, and withdrawing the whole of the evaporative medium entering the chamber at a point substantially at least as near the spinning end of the chamber as the point at which said introduction of evaporative medium is effected.
- 45 5. A process for the production of artificial filaments comprising extruding a spinning solution into a spinning chamber, introducing, from a side of said chamber, evaporative medium into the immediate vicinity of the filaments substantially at the point of extrusion, and withdrawing at least part of the evaporative medium entering the chamber at a point substantially at least as near the spinning end of the chamber as the point at which said introduction of evaporative medium is effected.
- 50 6. A process for the production of artificial filaments comprising extruding a spinning solution of a cellulose derivative into a spinning chamber, introducing evaporative medium into the immediate vicinity of the filaments substantially at the point of extrusion, and withdrawing at least part of the evaporative medium entering the chamber at a point substantially at least as near the spinning end of the chamber as the point at which said introduction of evaporative medium is effected.
- 55 7. A process for the production of artificial filaments comprising extruding a spinning solution of cellulose acetate into a spinning chamber, introducing evaporative medium into the immediate vicinity of the filaments substantially at the point of extrusion, and withdrawing at least part of the evaporative medium entering the chamber at a point substantially at least as near the spinning end of the chamber as the point at which said introduction of evaporative medium is effected.
- 60 8. A process for the production of artificial filaments comprising extruding a spinning solution downwardly into a spinning chamber, introducing evaporative medium into the immediate vicinity of the filaments substantially at the point of extrusion, and withdrawing at least part of the evaporative medium entering the chamber at a point substantially at least as near the upper end of the chamber as the point at which said introduction of evaporative medium is effected.
- 65 9. Process for the production of artificial filaments from solutions of organic derivatives of cellulose, said process comprising extruding a spinning solution into a current of evaporative medium, causing said current to flow in a direction opposite to the direction of extrusion of the filaments and introducing additional evaporative medium into the said current in the vicinity of the point of extrusion of the filaments.

10. Process for the production of artificial filaments from solutions of cellulose esters, said process comprising extruding a spinning solution into a current of evaporative medium, causing said current to flow in a direction opposite to the direction of extrusion of the filaments and introducing heated evaporative medium into the said current in the vicinity of the point of extrusion of the filaments. 80
11. Process for the production of artificial filaments from solutions of cellulose acetate, said process comprising extruding a spinning solution into a current of evaporative medium, causing said current to flow in a direction opposite to the direction of extrusion of the filaments and introducing additional evaporative medium into the said current in the vicinity of the point of extrusion of the filaments. 85
12. Process for the production of artificial filaments from solutions of organic derivatives of cellulose, said process comprising extruding a spinning solution into a current of evaporative medium, causing said current to flow in a direction opposite to the direction of extrusion of the filaments, introducing additional evaporative medium into said current in the vicinity of the point of extrusion of the filaments; and directing the said evaporative medium towards the filaments. 90
13. Process for the production of artificial filaments from solutions of organic derivatives of cellulose, said process comprising extruding a spinning solution into a current of evaporative medium, causing said current to flow in a direction opposite to the direction of extrusion of the filaments, and introducing additional evaporative medium into the said current at a point in proximity to the filaments immediately after they have left the point of extrusion. 95
14. Process for the production of artificial filaments from solutions of cellulose acetate, said process comprising extruding a spinning solution into a current of evaporative medium, causing said current to flow in a direction opposite to the direction of extrusion of the filaments, and introducing additional evaporative medium into the said current at a point in proximity to the filaments immediately after they have left the point of extrusion; and in a manner which is symmetrical with respect to the filaments. 100
15. Process for the production of artificial filaments from solutions of organic derivatives of cellulose, said process comprising extruding a spinning solution into a current of evaporative medium, causing said current to flow in a direction opposite to the direction of extrusion of the filaments, and introducing additional evaporative medium together with a proportion of vapors of a material which is a solvent for the substance of the filaments into the said current in the vicinity of the point of extrusion. 105
16. Process for the production of artificial filaments from solutions of organic derivatives of cellulose, said process comprising extruding the spinning solution downwardly into an upwardly moving current of evaporative medium, and introducing additional evaporative medium into the said current in the vicinity of the point of extrusion. 110
17. Process for the production of artificial filaments from solutions of organic derivatives of cellulose, said process comprising extruding a spinning solution into a current of evaporative medium, causing said current to flow in a direction opposite to the direction of extrusion of the filaments, and introducing additional evaporative medium into the said current in the vicinity of the point of extrusion. 115
18. Process for the production of artificial filaments from solutions of organic derivatives of cellulose, said process comprising extruding a spinning solution into a current of evaporative medium, causing said current to flow in controlled amount in a direction opposite to the direction of extrusion of the filaments, and introducing additional evaporative medium into the said current in the vicinity of the point of extrusion of the filaments. 80
19. Process for the production of artificial filaments from solutions of organic derivatives of cellulose, said process comprising extruding the spinning solution downwardly into a current of evaporative medium flowing upwardly in controlled amount, and introducing additional evaporative medium in controlled amount into the said current in the vicinity of the point of extrusion. 85
20. Process for the production of artificial filaments from solutions of cellulose esters, said process comprising extruding a spinning solution downwardly into a current of evaporative medium flowing upwardly in controlled amount, and introducing additional evaporative medium in controlled amount into the said current in the vicinity of the point of extrusion of the filaments. 90
21. Process for the production of artificial filaments from solutions of cellulose acetate, said process comprising extruding a spinning solution downwardly into a current of evaporative medium, flowing upwardly in controlled amount and introducing additional evaporative medium in controlled amount into the said current in the vicinity of the point of extrusion of the filaments. 95
22. Dry-spinning apparatus for the production of artificial filaments, said apparatus comprising a spinning chamber, a spinning jet disposed near an end of said chamber, means for introducing evaporative medium into the immediate vicinity of said jet, and means for withdrawing evaporative medium from the chamber, said means being disposed substantially as near the spinning end of the chamber as the said introducing means. 100
23. Dry-spinning apparatus for the production of artificial filaments, said apparatus comprising a spinning chamber, a spinning jet disposed near an end of said chamber, means for introducing evaporative medium into the immediate vicinity of said jet, means for withdrawing evaporative medium from the chamber, said means being disposed substantially as near the spinning end of the chamber as the said introducing means, and means for introducing evaporative medium into the chamber at the end remote from the jet. 105
24. Dry-spinning apparatus for the production of artificial filaments, said apparatus comprising a spinning chamber, a spinning jet disposed near an end of said chamber, means for introducing evaporative medium into the immediate vicinity of said jet, and means for withdrawing evaporative medium from the chamber, said means being disposed at one side of the chamber at a point substantially as near the spinning end of the chamber as the said introducing means. 110
25. Dry-spinning apparatus for the production of artificial filaments, said apparatus comprising a spinning chamber, a spinning jet disposed near an end of said chamber, means at a side of the jet for introducing evaporative medium into the im- 115

mediate vicinity of said jet, and means for withdrawing evaporative medium from the chamber, said means being disposed substantially as near the spinning end of the chamber as the said introducing means.

5 26. Dry spinning apparatus for the production of artificial filaments, said apparatus comprising a spinning chamber, a spinning jet disposed in said chamber, means for causing a current of evaporative medium to pass through the said chamber in a direction opposite to the direction of extrusion of the filaments, and means for introducing additional evaporative medium into the said current in the vicinity of the jet.

10 27. Dry spinning apparatus for the production of artificial filaments, said apparatus comprising a spinning chamber, a spinning jet disposed in said chamber, means for causing a current of evaporative medium to pass through the said chamber in a direction opposite to the direction of extrusion of the filaments, and a perforated tubular ring adapted to introduce additional evaporative medium into the said current in the vicinity of the jet, said perforated tubular ring being 15 symmetrically disposed with reference to the jet.

20 28. Dry spinning apparatus for the production of artificial filaments, comprising a spinning chamber, a spinning jet disposed in the upper end of said chamber, means for causing a current

30

of evaporative medium to pass upwardly through the said chamber, and means for introducing additional evaporative medium into the said current in the vicinity of the spinning jet.

29. Dry spinning apparatus for the production of artificial filaments, said apparatus comprising a spinning chamber, a spinning jet disposed in said chamber, means for causing a current of evaporative medium to pass through the said chamber in a direction opposite to the direction of extrusion of the filaments, means for introducing additional evaporative medium into the said current in the vicinity of the jet and means for controlling the amount of additional evaporative medium so introduced.

30. Dry spinning apparatus for the production of artificial filaments, said apparatus comprising a spinning chamber, a spinning jet disposed in said chamber, means for causing a current of evaporative medium to pass through the said chamber in a direction opposite to the direction of extrusion of the filaments, means for controlling the amount of evaporative medium passing through the chamber, and means for introducing additional evaporative medium into the said current in the vicinity of the jet.

JOHN FREDERICK BRIGGS.  
ROBERT PIERCE ROBERTS.

80

85

90

95

100

105

110

35

40

115

45

120

50

125

55

130

60

135

65

140

70

145

75

150